

Patented Oct. 10, 1939

2,175,212

UNITED STATES PATENT OFFICE

**2,175,212**

## **MANUFACTURE OF SMOKELESS POWDER**

**Fredrich Olsen, Gordon C. Tibbitts and Edward B. W. Kerone, Alton, Ill., assignors to Western Cartridge Company, East Alton, Ill., a corporation of Delaware**

**No Drawing. Application July 10, 1935,  
Serial No. 30,634**

**6 Claims. (Cl. 52—20)**

This invention relates generally to the manufacture of explosives and particularly to a process of manufacturing propellant powder from deteriorated nitrocellulose powder as the raw material and pertains particularly to purification and stabilization of such deteriorated nitrocellulose to an extent sufficient to adapt it for use as a propellant.

10 Nitrocellulose in general and cannon powder in particular decompose in spots. These spots are centers of high acid content and contain no un-nitrated diphenylamine to absorb the acid which is being liberated. Furthermore, while diphenylamine is a neutral amine, its nitration products 15 nitrosodiphenylamine, nitrodiphenyl amine, di-nitrodiphenylamine and trinitrodiphenylamine are acidic, and in large quantities, such as are present in one of these spots, may be antagonistic toward nitrocellulose. Various decomposition 20 products such as ether peroxide formed by oxidation of the residual ether, ethyl nitrate formed by alcoholysis of the nitrocellulose by the residual alcohol, and the possible presence of cellulose nitrite would help explain the unstable character 25 of some cannon powders.

25 The object of the present invention, generally stated, is to provide a process of purifying unstable or partially decomposed nitrocellulose to an extent sufficient to adapt it for use as a propellant.

30 A further object of this invention is to provide a process of treating deteriorated nitrocellulose containing centers of high acid concentrations whereby to disperse the acid and render the  
35 nitrocellulose suitable for use.

35 A more specific object of this invention is to provide a process for reclaiming deteriorated cannon powder wherein the centers of high acid concentration are dispersed, utilized and washed out to an extent sufficient to adapt the nitrocel-  
40 lulose for use as a propellant.

Other objects will become apparent to those skilled in the art when the following description is read.

45 In accordance with this invention, generally stated, nitrocellulose which has deteriorated or contains centers of high acid concentration, as is frequently present in aged cannon powder, may be purified and stabilized to an extent sufficient  
50 to render it suitable for use as a propellant. This may be conveniently accomplished, in accordance with one embodiment of this invention, by grinding the deteriorated nitrocellulose powder, as for instance in a water slurry, and thereafter agitating the slurry in a sufficient quantity of a vehicle,

such as water, to wash out and disperse the centers of high acidity. It is also desirable to add to the slurry a sufficient quantity of a neutralizing agent, such as calcium carbonate or other mild alkali, so as to neutralize the acid which may be washed out of the comminuted nitrocellulose. In order to facilitate distribution and liberation of the nitrated centers, which may consist of nitrated diphenylamine, the deteriorated nitrocellulose may be softened as by treatment with a suitable solvent and this may even be carried out to the extent of forming a lacquer solution as described in our copending application Serial No. 598,332 now Patent No. 2,027,114 granted January 7, 1936, where the lacquer is made using a solvent for nitrocellulose which is substantially immiscible with water, for instance, ethyl acetate. By this action the nitric acid present in the spots is liberated and spread uniformly throughout the bath of water. This is important since a small amount of acid uniformly distributed through nitro-cellulose might not be harmful, whereas this same quantity of acid when locally concentrated would be injurious. The acidic nitrated diphenylamines are also brought into homogeneous solution, and diphenylamine which could not be reached by the nitric acid is brought into intimate contact therewith. More diphenylamine is usually added to the solution as a further safeguard.

In accordance with this invention, therefore, the series of purifying steps may include grinding and washing only, softening and washing only or the combination of grinding (with or without subsequent washing) and softening and washing.

When the softened dissolved, or partially dissolved or gelatinized nitrocellulose is washed with water containing calcium carbonate, acid diffuses out of the nitrocellulose into the water and is neutralized. This alkaline medium also has a hydrolyzing action upon any unstable esters which may be present and the solvent action of the water frees the solution of ether peroxide if such is present.

A mild alkaline material like calcium carbonate was chosen for the following reasons: When calcium carbonate is suspended in water some of it dissolves setting up the following equilibrium: 45



The concentration of OH ion is large enough to neutralize acids (which shifts the equilibrium to the right) but not large enough to injure the nitrocellulose. As soon as some of the OH ions 55

are neutralized, more undissolved calcium carbonate dissolves and hydrolyzes.

Sufficient fresh diphenylamine may then be added to the softened nitrocellulose in order to compensate for that portion of the diphenylamine previously present which has become nitrated and been diffused or liberated by the reclaiming process of the present invention. In order to accomplish this, fresh diphenylamine may be incorporated with the solvent with which the deteriorated nitrocellulose is first softened, or may be applied in a suitable manner after the washing and neutralization is completed.

As an illustrative embodiment of the present invention, grains of completely gelatinized, but partially deteriorated nitrocellulose cannon powder, which contain unstable regions, may be finely divided in a suitable machine, such for instance, as by a beater. This grinding may be carried out in buffered water of a pH value above 7.2 until the material is fine enough to pass, for instance, an 80 mesh screen. This treatment concurrently comminutes and washes the powder, and alone accomplishes a noticeable improvement in the stability of the powder.

Further improvements in the stability, however, may be accomplished by carrying out either of the processes of graining described and claimed in our prior copending applications Serial No. 30 598,332, filed March 12, 1932, and Serial No. 620,302, filed June 30, 1932 with sufficient of an alkaline substance, such as calcium carbonate, in the water of the graining bath to neutralize the acid which may be liberated or washed out of the 35 nitrocellulose during the graining process. In the case of the former application the nitrocellulose lacquer is washed by agitation in the water bath while in the latter case softened nitrocellulose particles are similarly washed. As to common subject matter this application may be regarded as a continuation in part of said prior applications Serial No. 598,332 now Patent No. 2,027,114, and Serial No. 620,302.

As a further example, freshly nitrated nitrocellulose which is to be dissolved, gelatinized, or even softened to form grains may be purified by washing the lacquer or softened nitrocellulose as above described. For instance, if gun cotton or nitrated wheat straw paper is used as the 50 raw material in the process of application Serial No. 598,332, the final washing stages of the usual nitration process may be omitted. Hence the bulk nitrocellulose after nitration and having only one or two washings is still in a more or 55 less impure condition, but in this condition it may be dissolved, or merely softened, by the action of a solvent and washed. Of course, if free nitric acid is present in the softened or dissolved 60 nitrocellulose the washing water may be made mildly alkaline, as by the addition of calcium carbonate as above described. Accordingly, final purification of fresh nitrocellulose is thereby ac-

complished concurrently with the graining operation.

From the foregoing description it is apparent that many modifications of the process hereinbefore described will present themselves to those skilled in the art without departing from the spirit of this invention. It is to be distinctly understood, therefore, that the embodiments hereinbefore described are merely illustrative of the procedure which may be followed but that the invention is not limited thereto. Such modifications and the use of such individual features and such subcombinations of features as do not depart from the spirit of this invention are, although not specifically described hereinbefore, contemplated by and within the scope of the appended claims.

Having thus described the invention, what is claimed is:

1. In the art of treating deteriorated nitrocellulose containing regions of acid concentration, the process comprising, softening the nitrocellulose with a solvent therefor, which is immiscible with water, and washing the solution in a bath of water.

2. In the art of treating deteriorated nitrocellulose containing regions of acid concentration, the process comprising, softening the nitrocellulose with a solvent therefor, washing the softened nitrocellulose in a mildly alkaline bath, 30 and adding additional stabilizer while the nitrocellulose is soft.

3. In the art of purifying nitrocellulose the process comprising, treating nitrocellulose containing acidic impurities with a solvent for nitrocellulose until softened or dissolved, and washing the nitrocellulose while thus softened or dissolved in a mildly alkaline bath in a bath in which the solvent is immiscible.

4. In the art of treating impure nitrocellulose, 40 the process comprising, treating the nitrocellulose with a solvent therefor until the nitrocellulose is dissolved, said solvent being substantially immiscible with water, and agitating the solution in a bath of water sufficiently alkaline 45 to neutralize acid washed from the nitrocellulose solution.

5. In the art of treating deteriorated nitrocellulose containing ingredients which tend to produce acidic impurities, the process comprising, 50 softening the nitrocellulose with a solvent therefor which is immiscible with water, and washing the solution in a bath of water.

6. In the art of purifying nitrocellulose the process comprising, treating nitrocellulose containing ingredients tending to produce acidic impurities with a solvent for nitrocellulose until softened or dissolved, and washing the nitrocellulose while thus softened or dissolved in a mildly 60 alkaline bath in which the solvent is immiscible.

FREDRICH OLSEN.

GORDON C. TIBBITS.

EDWARD B. W. KERONE.

CERTIFICATE OF CORRECTION.

Patent No. 2,175,212.

October 10, 1939.

FREDRICH OLSEN, ET AL.

It is hereby certified that error appears in the printed specification of the above numbered patent requiring correction as follows: Page 2, second column, line 38, claim 3, strike out the words "in a bath"; and that the said Letters Patent should be read with this correction therein that the same may conform to the record of the case in the Patent Office.

Signed and sealed this 16th day of January, A. D. 1940.

(Seal)

Henry Van Arsdale,  
Acting Commissioner of Patents.